# EUROPEAN PATENT SPECIFICATION

(11) **EP 2 481 825 B1**
(45) Date of publication and mention of the grant of the patent: **08.05.2013**
(21) Application number: 11152827.9
(22) Date of filing: 01.02.2011
(51) Int. Cl.: C22C 23/04, C22C 23/06

(54) **Magnesium alloy containing rare earth metals**
Seltenerdmetalle enthaltende Magnesiumlegierung
Alliage de magnésium contenant des métaux de terres rares

(43) Date of publication of application: 01.08.2012
(73) Proprietor: Helmholtz-Zentrum Geesthacht Zentrum für Material- und Küstenforschung GmbH, 21502 Geesthacht (DE)
(72) Inventor: Huang, Yuanding, 21502 Geesthacht (DE); Peng, Qiuming, 066004, Quinhuangdao (CN); Hort, Norbert, 21339 Lüneburg (DE); Kainer, Karl Ulrich, 21522 Hohnstorf (DE)
(74) Representative: UEXKÜLL & STOLBERG

(56) References cited:
- WO-A1-2004/001087
- WO-A1-2006/125278
- WO-A1-2009/039581
- WO-A1-2009/086585
- SUDHOLZ, A. D. ET AL: "Unraveling the corrosion properties of magnesium rare earth alloys", MAGNESIUM, INTERNATIONAL CONFERENCE ON MAGNESIUM ALLOYS AND THEIR APPLICATIONS, 8TH, WEIMAR, GERMANY, OCT. 26-29, 2009 , MEETING DATE 2009, 866-871. EDITOR(S): KAINER, KARL ULRICH. PUBLISHER: WILEY-VCH VERLAG GMBH & CO. KGAA, WEINHEIM, GERMANY. CODE, 2010, XP009157828,
- YAMADA KENTARO ET AL: "Precipitate microstructures of high strength Mg-Gd-Y- Zn - Zr alloys", 1 January 2006 (2006-01-01), ADVANCED MATERIALS RESEARCH,, PAGE(S) 417 - 420, XP009092939, ISSN: 1022-6680
- HONMA ET AL: "Effect of Zn additions on the age-hardening of Mg-2.0Gd-1.2Y-0.2Zr alloys", ACTA MATERIALIA, ELSEVIER, OXFORD, GB, vol. 55, no. 12, 8 June 2007 (2007-06-08), pages 4137-4150, XP022110797, ISSN: 1359-6454, DOI: 10.1016/J.ACTAMAT.2007.02.036

## Description

### FIELD OF THE INVENTION

The present invention relates to cast and wrought single-phase solid solution magnesium alloys with high mechanical properties, formability and corrosion resistance.

### BACKGROUND

Magnesium alloys have not yet been widely accepted by car manufacturers. Most of the technical barriers preventing magnesium alloys from widespread applications arise from the low ductility and toughness at low temperatures, poor corrosion and creep resistance at high temperatures. Their present commercial products are normally fabricated by high pressure die casting. The use of wrought magnesium alloys is limited because of its poor formability and corrosion resistance.

It will be necessary to improve the low-temperature formability of wrought magnesium alloys in order to obtain a higher acceptance of these alloys in industry. Low ductility and low toughness are due to the intrinsically brittle nature of the hexagonal close-packed crystal structure. A further issue which hinders the acceptance of wrought magnesium alloys is their poor corrosion resistance.

Most commercial wrought magnesium alloys belong to magnesium-aluminium (Mg-Al) and magnesium-zinc (Mg-Zn) series. The later developed magnesium-rare earth (Mg-RE) series such as WE43 (Mg-4.1Y-2.2Nd-1HRE-0.5Zr) and WE54 (Mg-5.2Y-1.7Nd-1.7HRE-0.4Zr) alloys were not accepted by the industry due to their high price arising from the high content of rare earth elements.

The documents:
YAMADA KENTARO ET AL: "Precipitate microstructures of high strength Mg-Gd-Y-Zn-Zr alloys", 1 January 2006, ADVANCED MATERIALS RESEARCH, pages 417- 420, ISSN: 1022-6680
   and
HONMA ET AL: "Effect of Zn additions on the age-hardening of Mg-2.0Gd-1.2Y-0.2Zr alloys", ACTA MATERIALIA, ELSEVIER, OXFORD, GB, vol. 55, no. 12, 8 June 2007, pages 4137-4150, ISSN: 1359-6454
disclose magnesium alloys containing Gd and Y.

The alloys of magnesium-aluminium series are the most commonly used in wrought applications for their relative ease of extrusion and adequate mechanical properties, but they suffer from both a pronounced asymmetry in the yield behaviour and a relatively narrow processing window. Due to the lower eutectic temperature 437°C for magnesium-aluminium alloys, the hot processing temperatures are normally selected below 350°C and the processing speeds are not so high. If selecting high temperatures more than 350°C with high processing speeds, the eutectic phases dissolve again, leading to the occurrence of hot cracking and bad surface quality of the products. In addition, until now, the methods for refining the as-cast microstructures of magnesium-aluminium alloys are not satisfying and not widely accepted by the industry.

Since magnesium-zinc series contain no aluminium, their as-cast microstructure can be effectively refined by the addition of zirconium. However, these magnesium-zinc alloys still have very limited applications because they are susceptible to microporosity during casting. The addition of zinc in magnesium increases the susceptibility to hot tearing. Moreover, due to the high content of zinc, it was considered that these alloys are difficult to be welded.

Therefore, at present only AZ31 (Mg-2.9Al-0.8Zn) alloy is used in industry to an significant extent. However, AZ31 (Mg-2.9Al-0.8Zn) alloy exhibits some problems with recrystallisation during the hot working and has insufficient mechanical and corrosion properties.

It is therefore the object of the present invention to develop new magnesium alloys with high corrosion resistance and formability using innovative alloy design concept.

### SUMMARY OF THE INVENTION

Accordingly, the present invention provides a magnesium alloy as defined in claim 1.

### DETAILED DESCRIPTION OF THE INVENTION

The strengthening effects of rare earths in the previous magnesium alloys have been explained by two mechanisms, precipitate strengthening and solid solution strengthening. Precipitate strengthening, especially the age hardening, has been emphasised to improve the mechanical properties. Without being bound to any theory, it is believed that in alloys of the present invention, precipitate strengthening is avoided and that solid solution strengthening is the main mechanism which improves the mechanical properties in the magnesium alloys according to the present invention.

It is further believed that the solid solution strengthening depends on the contents of alloying elements in the matrix of magnesium and the difference in atomic radius between the alloying elements and magnesium such that a high content of alloying elements and large difference in atomic radius increase the effect of solid solution strengthening.

In addition, it has been found that there exists a synergistic effect caused by the interaction of the different rare earth elements. With the same total content of rare earth elements in the magnesium alloy, the improvement in mechanical properties is higher when two different rare earth elements are present in comparison to the improvement achieved with the presence of only on e rare earth element.

Furthermore, the addition of rare earth elements can purify the melt during casting. The addition of rare earth elements can remove impurity elements such as hydrogen, oxygen, chlorine, etc. Moreover, they interact with iron, cobalt, nickel or copper elements during melting, and these elements are removed by the formation of intermetallic compounds which settle at the bottom of the ingot. The decrease of impurities in the matrix also contributes to the high corrosion resistance.

Preferably, the magnesium alloy of the present invention further comprises an element selected from the group consisting of Zr, Ca, Zn, and mixtures thereof. The stress corrosion of magnesium alloys could be alleviated by the addition of zirconium (Zr) and rare earth elements. Zirconium (Zr) can be used as an element to decrease the stress corrosion cracking.

The magnesium alloys according to the present invention contain no aluminium; therefore, their as-cast microstructure can effectively be refined by the addition of zirconium or calcium.

In principle, two groups of rare earth elements can be classified in periodic table: light rare earth elements and heavy rare earth elements. In each group, rare earth elements have the similar chemical and physical properties. Due to the similar properties of yttrium and scandium to heavy rare earth elements, for the purposes of the present invention Y and Sc are treated as they were heavy rare earth elements. The light rare earth elements include samarium, lanthanum, cerium, neodymium, and praseodymium, and the heavy rare earth elements include gadolinium, yttrium and dysprosium. Besides the last three mentioned rare earth elements, zirconium and/or calcium are preferably added as a grain refiner.

The total content of rare earths is maintained below 5 wt.%, mainly for economical reasons. The content of grain refiner calcium and/or zirconium is preferably in the range of 0.05-0.6% by weight.

The manufacturing processes of the magnesium alloys according to the present invention are not restricted. The alloys can be prepared by die casting, permanent casting, chill casting, semi-solid processes, continuous casting or continuous twin roll casting.

The magnesium alloys according to the present invention exhibit excellent room temperature ductility with a value of about 25%.

Tensile tests show that as-cast alloy Mg0.4Gd0.4Y0.4Dy0.2Zr and Mg0.4Gd0.4Y0.4Dy0.2Zn0.2Zr exhibit excellent ductility. The elongation is more than 20%, which is much higher than that of AZ31 alloy. These two alloys have shown a good deformability.

### BRIEF DESCRIPTIONS OF THE DRAWINGS

The above and other characteristics and advantages of the invention will be more readily apparent through the following examples, and with reference to the appended drawings, where:
**Figure 1** compares the optical microstructure of the investigated, as cast alloys ((a) Mg, (b) Mg-0.4Y, (c) Mg-0.4Gd-0.4Y, (d) Mg-0.4Gd-0.4Y-0.4Dy, (e) Mg-0.4Gd-0.4Y-0.4Dy-0.2Zr, (f) Mg-0.4Gd-0.4Y-0.4Dy-0.2Zn, (g) Mg-0.4Gd-0.4Y-0.4Dy-0.2Ca, (h) Mg-0.4Gd-0.4Y-0.4Dy-0.2Zn-0.2Zr and (I) AZ31);
**Figure 2** shows the grain size, hardness and corrosion properties of the investigated alloys;
**Figure 3** shows the tensile properties of selected as-cast alloys; and
**Figure 4** shows the microstructural situation and the micro-segregation of the alloying elements.

### EXAMPLES

Three rare earth elements gadolinium, yttrium, dysprosium with high solubility in magnesium were selected to develop the single-phase solid solution magnesium alloys. Table 1 lists the compositions of the investigated alloys. A conventional alloy, Mg-3Al-1Zn (AZ31), was included for comparison.

All alloys were prepared by zone solidification. Their optical microstructures are shown in Figure 1. The average grain size decreases with the increment in the content of rare earths. Compared to the gadolinium and dysprosium, the yttrium element is the most effective element to decrease the grain size. The average grain sizes of E and H alloys containing zirconium are 55 µm and 67 µm. The average grain size of Mg-3Al-1Zn (AZ31 is 480 µm.

**Table 1. Nominal compositions of the investigated alloys**

| Alloys | (Composition (weight percent, wt.%) | | | | | | | |
|---|---|---|---|---|---|---|---|---|
| | Mg | Gd | Y | Dy | Zn | Al | Zr | Ca |
| A-Pure Mg | 100 | - | - | - | - | - | - | |
| B-Mg0.4Y | Bal* | - | 0.4 | - | - | - | - | |
| C-Mg0.4Gd0.4 Y | Bal | 0.4 | 0.4 | - | - | - | - | |
| D-Mg0.4Gd0.4 Y0.4Dy | Bal | 0.4 | 0.4 | 0.4 | - | - | - | |
| E-Mg0.4Gd0.4Y0.4DyO.2Zr | Bal | 0.4 | 0.4 | 0.4 | - | - | 0.2 | |
| F-Mg0.4Gd0.4 Y0.4Dy0.2Zn | Bal | 0.4 | 0.4 | 0.4 | 0.2 | | | |
| G-Mg0.4Gd0.4 Y0.4Dy0.2Ca | Bal | 0.4 | 0.4 | 0.4 | | | | 0.2 |
| H-Mg0.4Gd0.4 | Bal | 0.4 | 0.4 | 0.4 | 0.2 | - | 0.2 | |
| Y0.4Dy0.2Zn0.2Zr | | | | | | | | |
| I-AZ31 | Bal | - | - | - | 1.0 | 3.0 | - | |

| | | | | | | | | |
|---|---|---|---|---|---|---|---|---|
| * Balance. | | | | | | | | |

## Claims

1. A magnesium alloy consisting of (a) Mg; (b) 0.5 wt.% to less than 5.0 wt.% of at least two elements selected from the group consisting of Y, Gd, and Dy; and (c) optionally Zr, Ca and/or Zn; wherein the content, based on the total weight of the alloy, of each of said elements Y, Gd, and Dy, if present, is from 0.05 to 2.0 % by weight; and wherein the content, based on the total weight of the alloy, of each of said elements selected from the group consisting of Zr, Ca and Zn, if present, is from 0.05 to 0.6 wt.%; the remainder being magnesium.

2. A magnesium alloy according to any of the previous claims, wherein Gd is present in an amount by weight of 0.05 to 2.0 %.

3. A magnesium alloy according to any of the previous claims, wherein Y is present in an amount by weight of 0.05 to 2.0 %.

4. A magnesium alloy according to any of the previous claims, wherein Dy is present in an amount by weight of 0.05 to 2.0 %.

5. A magnesium alloy according to any of the previous claims, wherein Ca is present in an amount by weight of 0.05 to 0.4 %.

6. A magnesium alloy according to any of the previous claims, wherein Zr is present in an amount by weight of 0.2 to 0.6 %.

7. Use of the magnesium alloys according to any of claim 1 to 9 as casting magnesium alloys, wrought magnesium alloys, or degradable biomaterials.

## Patentansprüche

1. Magnesiumlegierung bestehend aus (a) Mg; (b) 0,5 Gew.% bis weniger als 5,0 Gew.% von mindestens zwei Elementen, die aus der Gruppe bestehend aus Y, Gd und Dy ausgewählt sind; und (c) gegebenenfalls Zr, Ca, und/oder Zn; wobei der Gehalt, auf Basis des Gesamtgewichts der Legierung, von jedem der Elemente Y, Gd und Dy, wenn vorhanden, von 0,05 bis 2,0 Gew.% beträgt; und wobei der Gehalt, auf Basis des Gesamtgewichts der Legierung, von jedem der Elemente ausgewählt aus der Gruppe bestehend aus Zr, Ca und Zn, wenn vorhanden, 0,05 bis 0,6 Gew.% beträgt, wobei der Rest Magnesium ist.

2. Magnesiumlegierung nach einem der vorgehenden Ansprüche, in der Gd in einer Menge von 0,05 Gew.% bis 2,0 Gew.% vorhanden ist.

3. Magnesiumlegierung nach einem der vorgehenden Ansprüche, in der Y in einer Menge von 0,05 Gew.% bis 2,0 Gew.% vorhanden ist.

4. Magnesiumlegierung nach einem der vorgehenden Ansprüche, in der Dy in einer Menge von 0,05 Gew.% bis 2,0 Gew.% vorhanden ist.

5. Magnesiumlegierung nach einem der vorgehenden Ansprüche, in der Ca in einer Menge von 0,05 Gew.% bis 0,4 Gew.% vorhanden ist.

6. Magnesiumlegierung nach einem der vorgehenden Ansprüche, in der Zr in einer Menge von 0,2 Gew.% bis 0,6 Gew.% vorhanden ist.

7. Verwendung der Magnesiumlegierungen gemäß einem der Anspruch 1 bis 6 als Gussmagnesiumlegierungen, Knetmagnesiumlegierungen oder abbaubare Biomaterialien.

## Revendications

1. Alliage de magnésium composé de (a) Mg ; (b) 0,5 % en poids à moins de 5,0 % en poids d'au moins deux éléments choisis parmi Y, Gd et Dy ; et (c) éventuellement Zr, Ca et/ou Zn, la proportion, par rapport au poids total de l'alliage, de chacun desdits éléments Y, Gd et Dy, éventuellement présent, étant de 0,05 à 2,0 % en poids, et la proportion, par rapport au poids total de l'alliage, de chacun desdits éléments choisis parmi Zr, Ca et Zn, éventuellement présent, étant de 0,05 à 0,6 % en poids, le reste étant du magnésium.

2. Alliage de magnésium selon la revendication 1, dans lequel Gd est présent à raison de 0,05 à 2,0 % en poids.

3. Alliage de magnésium selon l'une quelconque des revendications précédentes, dans lequel Y est présent à raison de 0,05 à 2,0 % en poids.

4. Alliage de magnésium selon l'une quelconque des revendications précédentes, dans lequel Dy est présent à raison de 0,05 à 2,0 % en poids.

5. Alliage de magnésium selon l'une quelconque des revendications précédentes, dans lequel Ca est présent à raison de 0,05 à 0,4 % en poids.

6. Alliage de magnésium selon l'une quelconque des revendications précédentes, dans lequel Zr est présent à raison de 0,2 à 0,6 % en poids.

7. Utilisation des alliages de magnésium selon l'une quelconque des revendications 1 à 6 comme alliages de magnésium de fonderie, alliages de magnésium de forge ou biomatériaux dégradables.
